

1

2

2,758,943

## PROCESS OF SUPERFICIALLY SAPONIFYING A STRIP OF CELLULOSE ESTER

Roelof Jan Hendrik Alink, Johannes Cornelis Antonius Jaspers, and Tijs Willem van Rijssel, Emmasingel, Eindhoven, Netherlands, assignors to Hartford National Bank and Trust Company, Hartford, Conn., as trustee

No Drawing. Original application June 6, 1951, Serial No. 230,245, now Patent No. 2,704,262, dated March 15, 1955. Divided and this application January 13, 1955, Serial No. 481,714

Claims priority, application Netherlands June 6, 1950

5 Claims. (Cl. 117—62)

This invention relates to an improved method of making cellulosic film and more particularly to cellulosic films which are to be subsequently impregnated with a light-sensitive system containing a diazonium compound, and is a division of our co-pending application, Ser. No. 230,245, filed June 6, 1951, now U. S. Patent No. 2,704,262.

Fatty acid esters of cellulose films containing from 1.5 to 3.0 radicals of fatty acid per glucose unit were saponified in order to regenerate a cellulosic outer layer which can be readily impregnated with aqueous solutions. Such films had the undesirable feature that the outer layer swelled in aqueous solution while the unsaponified portion of the film did not swell, resulting in stresses in the film with subsequent peeling of the outer layer.

An object of the invention, therefore, is to provide a method to shrink the outer layer and to prevent its subsequent peeling.

This and further objects of my invention will appear as the specification progresses.

According to the invention, the cellulose strip after superficial saponification thereof is immersed in one or more after-treatment baths. One of the after-treatments contains an anti-peeling agent which shrinks an intermediate partially saponified layer such that upon subsequent immersion of the strip in an aqueous solution, for instance when impregnating the strip with a water-soluble light-sensitive system no stresses are created in the saponified layer which would cause it to peel from the underlying unsaponified portion of the strip.

The invention is particularly applicable to cellulose diesters which are subject to peeling after saponification. For example a fatty ester of cellulose containing more than 1.5 and less than 3.0 fatty acid radicals per glucose residue after superficial saponification, i. e. by immersion of a strip of this material in a saponifying bath for a given period of time to saponify at least one side of the strip to a desired depth, is immersed in a bath containing an anti-peeling agent which is capable of shrinking a layer intermediate the outer surface of the strip and the unsaponified portion of the strip which contains 0.5 to 1.5 fatty acid radicals per glucose residue.

Anti-peeling agents suitable for the aforesaid purposes are: primary saturated alcohols having a main chain of from 4 to 11 carbon atoms, such as butanol-1; a mixture of about one part of butanol-1 and about one part of either benzene or toluene; a mixture of about one part of butanol-1 and about one part of tetrahydronaphthalene; a mixture of about one part of butanol-1 and about one part of diethyl ether; a solution of about 1.5 n phosphoric acid and butanol-1.

Cellulosic films which initially contain ester plasticisers such as triphenylphosphate and tricresylphosphate, which upon the superficial saponification of the fatty acid cellulose ester are not saponified completely. Particularly the intermediate layer may hold or subsequently attract from the substratum by diffusion a comparatively large

amount of plasticiser resulting in deposition or turbidity of particles of plasticiser on the surface of the film, foil or the like. It has now been found that the plasticiser still present after saponification in the totally saponified layer and the intermediate layer of the foil, film or the like can be removed with the use of solvents. Such solvents are, for example, solutions of so-called "dispersion agents," such as a salt of a sulphated hydroxycarbonic acid having at least 10 carbon atoms, for example, ammonium or sodium salts of ricinolic acid esterified with sulphuric acid, in addition sodium oleate, the sodium salt of p-octylbenzenesulphonic acid, cationogenous dispersion agents such as dodecylaminehydrochloride or compounds derived therefrom and in addition non-ion forming dispersion agents, such as polyethers, derived from methylene or ethylene oxide, which at the end of the chain, are esterified, for example, with a lauryl alcohol. Solutions of from 5 to 10% by weight of these ion-forming dispersion agents in water are suited to free from plasticiser saponified superficial layers of foils, films or the like made of fatty acid cellulose esters.

An after-treatment bath may contain both an anti-peeling agent for partially esterified cellulose containing from 0.5 to 1.5 radicals of fatty acid per glucose residue and a solvent for the plasticiser. It must be noted that a great number of non-ion-forming shrinking agents also have a dissolving effect on plasticisers.

Since the intermediate layer formed during saponification does not swell appreciably in the solution of the dispersion agent there is no probability of the saponified layer peeling from the non-saponified substratum. There is therefore entire liberty in regard to the choice between treating the foil, film or the like upon saponification first with the use of the dispersion agent or by treating it first with the use of the anti-peeling agent. For the sake of simplicity the shrinking agent and the solvent for the plasticiser may be combined in one after-treatment bath.

The invention will now be described in connection with the following examples:

## Example I

A mechanically moved web 130  $\mu$  thick and made of cellulose acetate containing about 2.3 radicals of acetic acid per glucose unit is saponified at 24° C. for 45 seconds on two sides in a solution of 1 n potassium hydroxide in a mixture of 66 parts by volume of methanol and 34 parts by volume of water, shrinking then taking place for a period of 45 seconds in a mixture of 1 part by volume of butanol-1 and 1 part by volume of toluene. The web then passes during a period of 45 seconds through a stopper bath of 0.6 n acetic acid in butanol-1. Eventually the web is washed in circulating water for 2.5 minutes and after spraying with water and skimming dried with the use of warm air of about 90 to 100° C.

The thickness of the regenerated cellulose layer is 10  $\mu$  and that of the intermediate layer 4  $\mu$ . The adhesion of the saponified layer to the non-saponified substratum is excellent. The butanol-toluene mixture may be replaced with equally satisfactory results by a mixture of butanol-1 with benzene or with tetrahydronaphthalene or with diethyl-ether.

## Example II

A web 140  $\mu$  thick and made of cellulose acetate having an acetic acid content of 53.3% is passed mechanically at 23.5° C. at the rate of 60 seconds per bath in succession through the following baths:

- (a) 1-n potassium hydroxide in 66% methanol
- (b) Butanol-1
- (c) Ditto
- (d) 2 n phosphoric acid in water
- (e) Circulating water
- (f) Ditto,

use being made with advantage of the difference in specific gravity between butanol-1 and water so that the film upon immersion in bath (d) repels the alcohol.

The web is then sprayed with water for 30 seconds and after skimming at 90° C. dried with a warm flow of air. The thickness of the regenerated cellulose layer is 10  $\mu$  and that of the intermediate layer 3  $\mu$ . The adhesion of the saponified layer to the substratum is excellent.

*Example III*

Cellulose diacetate foil was superficially saponified for 1 minute in a solution of 1 n-potassium hydroxide in a mixture of 2 parts by volume of methanol and 1 part by volume of water at 25° C. The web was then immediately inserted in a solution obtained by diluting 10 ccs. of 89% phosphoric acid with 300 ccs. of butanol-1 (this solution is about 1.5 n). After immersion in this bath for 1 minute at 25° C. the foil was rinsed in water for 30 minutes and then dried in air. The saponified layer adheres most satisfactorily and the surface is smooth. It is preferred that the concentration of phosphoric acid should not be excessive since otherwise the surface of the saponified layer, which in itself is readily adhesive, tends to become slightly shrivelled.

While the invention has been described with reference to specific examples and applications thereof, other modifications will be readily apparent to those skilled in the art without departing from the spirit and scope of the invention as defined in the appended claims.

What we claim is:

1. A process of superficially saponifying a strip of cellulose ester containing between 1.5 and 3.0 radicals of fatty acid per glucose residue, which comprises the steps of immersing said strip in a saponifying bath containing at least 0.1 normal solution of an alkali hydroxide and an alcoholic solvent to effect rapid saponification of said strip for a time sufficient to produce a partially saponified layer in said strip containing between 0.5 and 1.5 fatty acid radicals per glucose residue, and thereafter immersing said strip for at least 45 seconds in butanol-1.

2. A process of superficially saponifying a strip of cellulose ester containing between 1.5 and 3.0 radicals of fatty acid per glucose residue, which comprises the steps of immersing said strip in a saponifying bath containing at least 0.1 normal solution of an alkali hydroxide and

an alcoholic solvent to effect rapid saponification of said strip for a time sufficient to produce a partially saponified intermediate layer in said strip containing between 0.5 and 1.5 fatty acid radicals per glucose residue, and thereafter immersing said strip for at least 45 seconds in a mixture of about one part of butanol-1 and about one part of a component having the formula  $C_nH_{(2n-6)}$ , where  $n$  is one of the integers 6 and 7.

3. A process of superficially saponifying a strip of cellulose ester containing between 1.5 and 3.0 radicals of fatty acid per glucose residue, which comprises the steps of immersing said strip in a saponifying bath containing at least 0.1 normal solution of an alkali hydroxide and an alcoholic solvent to effect rapid saponification of said strip for a time sufficient to produce a partially saponified intermediate layer in said strip containing between 0.5 and 1.5 fatty acid radicals per glucose residue, and thereafter immersing said strip for at least 45 seconds in a mixture of about one part of butanol-1 and about one part of tetrahydronaphthalene.

4. A process of superficially saponifying a strip of cellulose ester containing between 1.5 and 3.0 radicals of fatty acid per glucose residue, which comprises the steps of immersing said strip in a saponifying bath containing at least 0.1 normal solution of an alkali hydroxide and an alcoholic solvent to effect rapid saponification of said strip for a time sufficient to produce a partially saponified intermediate layer in said strip containing between 0.5 and 1.5 fatty acid radicals per glucose residue, and thereafter immersing said strip for at least 45 seconds in a mixture of about one part of butanol-1 and about one part of diethyl ether.

5. A process of superficially saponifying a strip of cellulose ester containing between 1.5 and 3.0 radicals of fatty acid per glucose residue, which comprises the steps of immersing said strip in a saponifying bath containing at least 0.1 normal solution of an alkali hydroxide and an alcoholic solvent to effect rapid saponification of said strip for a time sufficient to produce a partially saponified intermediate layer in said strip containing between 0.5 and 1.5 fatty acid radicals per glucose residue, and thereafter immersing said strip for at least 60 seconds in a solution of about 1.5 n phosphoric acid in butanol-1.

No references cited.